

# UNITED STATES PATENT OFFICE.

DAVID JOHNSON, OF SOUTH HAMPSTEAD, COUNTY OF MIDDLESEX,  
ENGLAND.

## PROCESS OF PREPARING EXPLOSIVES.

SPECIFICATION forming part of Letters Patent No. 376,000, dated January 3, 1888.

Application filed June 8, 1886. Serial No. 204,530. (No specimens.) Patented in England July 24, 1885, No. 8,951.

*To all whom it may concern:*

Be it known that I, DAVID JOHNSON, a subject of the Queen of Great Britain, residing at South Hampstead, in the county of Middlesex, 5 in England, have invented new and useful Improvements in the Manufacture of Explosives, (for which I have secured Letters Patent in Great Britain, No. 8,951, dated July 24, 1885,) of which the following is a specification.

The employment of nitro-cellulose, whether obtained by the nitration of cotton or of wood, or other analogous substances, in the preparation of powder for sporting and military fire- 15 arms, has hitherto been retarded by the uncertainty attendant upon the manufacture and use of such powder.

My invention provides simple, safe, cheap, and certain means for making, on a large scale, 20 sporting and military powders easy of ignition, but of any required hardness and density for slow combustion and maximum velocity with lowering of trajectory. In my process I use any nitro-cellulose compounds of various degrees of nitration, alone or in combination—such as trinitro, dinitro, and mononitro cellulose, and those of intermediate nitration, and also dinitro-cellulose alone or together with nitro-cellulose compounds of lower degrees of 25 nitration than trinitro-cellulose—viz., without trinitro-cellulose, as heretofore. The ordinary gun-cotton now used is an imperfect trinitro-cellulose, inasmuch as it contains proportions of other nitro-cellulose of lower degrees of nitration, which proportions practically are of a 30 varying quantity, so that it is difficult to obtain commercially two samples alike. Although these variations may be slight, yet in practice I have found by experiment that they 35 induce marked variable and sometimes dangerous effect in the action of the finished product when used in the fire-arm.

Where hereinafter I speak generally of trinitro-cellulose, it includes what is called "gun-cotton."

While I do not in my invention confine myself to the use of dinitro-cellulose alone or in admixture, yet I have found by experiment 45 that where gun-cotton or trinitro cellulose is used as one of the essential constituents of the

explosive, either in my invention or by the processes employed in the preparation of the various heretofore known nitro compounds, (used for fire-arms,) an element of uncertainty is introduced owing to the difficulty of preparing commercially a true trinitro-cellulose. 55 An element of great uncertainty is thus introduced into the explosive, which, under certain further slightly-varying conditions—such as manner of loading, pressure in loading, 60 strength of cap, and shape of cartridge-case—render it extremely difficult and almost impossible to prepare a powder for the above purposes which shall not, under some of these varying conditions, explode with abnormal 65 suddenness, and thus give rise to an abnormal strain upon the weapon, sometimes even to bursting force, as has often been the case in practice.

An element of danger has been discovered 70 in powders containing trinitro-cellulose in important quantities, as in powders made from nitro-cellulose now in the market, in regard to the amount of moisture contained in such powders. There appears in this respect to be 75 only one condition of maximum utility and of safety, and that is when the powder is in its average normal or air-dry state. When, however, such powder is subjected to extremely moist conditions, and consequently takes up 80 more moisture than its average normal or air-dry condition would demand, then there is objectionable "hang fire." This moisture can be driven off, and when the powder has regained 85 its average normal air-dry state, then it regains its usefulness; but if (as has been found the case in practice) the powder has been subjected to a warmth or heat sufficient to dry the powder below its average normal air-dry state, then abnormal variations in the explosive 90 force take place, varying in intensity according to the dryness, and up to complete dryness of the powder, in which state also experiment has proved powders containing trinitro cellulose to be exceedingly dangerous.

The powder manufactured by my process has the further advantage that if it should by any chance take up an excess of moisture over the average normal quantity, then, if such powder be subjected to warmth or heat 95

to drive off such excess of moisture, (even if the moisture be absolutely removed,) the strain upon the weapon set up by such dry powder is never more than that of ordinary black gunpowder in its ordinary shooting state, and the powder manufactured by my process exerts in its average normal or air-dry state a strain upon the weapon much less than that from ordinary gunpowder.

10 In powder prepared by my improved simple and commercial process of manufacture from nitro-cellulose of lower degrees of nitration than that of the trinitro compound there is regularity and certainty in the finished product; and slightly varying conditions—such as manner of loading, pressure in loading, strength of cap, shape of cartridge-case, and the varying amount of moisture in the powder—do not exert any marked or dangerous effect 15 in its use; and generally in the use of a powder prepared by my process there is a more gradual pressure during combustion in the gun than in the case of a powder yielding the same projecting force, but containing trinitro-cellulose 20 in important quantities, as in such powders now in the market.

In carrying my invention into effect the nitro compound mixed with sufficient water to be uninflammable—such, and for example, 25 as dinitro-cellulose—is first mixed, by appropriate means, with oxidizing agents, as nitrate of potassium or of barium, and when deemed advisable, according to the exact use to which the explosive is to be put, with other materials—such, for instance, as hydro-cellulose, wood-flour, torrefied starch, lamp-black, or charcoal. As an example, for military firearms, I may mention fifty parts, by weight, of nitro-cellulose, forty parts of nitrate of potassium, and ten parts of torrefied starch or lamp-black. As an example, for sporting and shot guns, I may mention fifty parts of nitro-cellulose, twenty-five parts of nitrate of barium, twenty-two parts of nitrate potassium, and three parts of torrefied starch or lamp-black. The nitro compound, either pure or in admixture with substances, such as are mentioned above, is then brought into the form of small granules, by well-known means, 45 or is molded by more or less compression into suitable forms—such, for instance, as cylinders, prisms, or cubes. The granular powder, hereinafter spoken of as the grains or the cylinders, prisms, or cubes, hereinafter described 50 as the blocks, are deprived of their moisture, by heat or otherwise, and are then fit to undergo the treatment about to be described. A weighted quantity of the grains or blocks is taken, and a preliminary experiment is made 55 to determine what quantity of any of the solvents or mixed solvents of camphor is required to saturate the grains or blocks without these being unduly wet. The solvent or mixed solvents of camphor chosen are such as evaporate 60 below 100° centigrade, and neither *per se* nor with the camphor in solution exert any material gelatinizing, solvent, or detrimental action

upon the explosive compound. In practice light petroleum or benzoline is found both an economical and convenient solvent for the camphor. Various non-volatile oils—such as paraffine-oil, rosin-oil, or easily-fusible fatty or resinous matters—may also be added to the grains or blocks, as I have found that such materials aid in effecting the desired slowing 75 action. This is easily and conveniently effected by introducing the same into the camphor solution, so that when the volatile solvent or solvents are driven off the non-volatile oily or fatty matter remains behind in the 80 grains or blocks, together with the camphor.

Having discovered the proper saturating proportions of the solvent or mixed solvents of camphor in relation to the grains or blocks, a solution of camphor is prepared, of a strength 85 such that the grains or blocks when saturated with the solution may contain that quantity of camphor which is found by experiment to effect the production, as may be desired, of an explosive more or less hard and, respectively, 90 of a more or less slowly-burning nature. In practice it is found that a proportion of one part, by weight, of camphor and five parts, by weight, of the solvent to ten parts, by weight, of the nitro compound or mixture gives good 95 results; but it is to be clearly understood that the proportion is not limited to this or any other herein expressed or unexpressed; or instead of the one part of camphor I may use, say, 0.5 part of camphor, five parts of the 100 solvent, and 0.5 part of phenol to ten parts, by weight, of the nitro compound or mixture. Having prepared an appropriate solution of camphor, the grains or blocks are saturated therewith, sufficient time being allowed for the 105 solution to thoroughly permeate every part of the nitro compound. The grains or blocks may be saturated with the camphor solution by pouring a regulated quantity of the solution upon the nitro compound and agitating 110 to effect proper admixture; or it may be effected by immersing the grains or blocks contained in a perforated basket of wire-gauze or other material in the camphor solution, either under reduced, or it may be, ordinary atmospheric pressures. In order to effect a more 115 intimate action or penetration in the pores, especially with large blocks, I may exhaust the air more or less from the space above the saturating-liquid contained in a closed vessel, 120 and from the pores of the nitro compound placed in that space before immersion, and admit the air again after immersion, so as to use the air-pressure to complete the saturation, suitable means being provided for lowering 125 and raising the basket into and out of the liquid while in the saturating-vessel. I then allow the excess of liquid adhering to the grains or blocks to drain off before proceeding with the next process—viz., that of evaporating off the volatile solvent and collecting the same for repeated use.

It is to be clearly understood that I do not bind myself to the employment of any special

form of apparatus for effecting the evaporation and condensation of the volatile solvent; but in practice I have found it convenient to employ a circular pan heated from without by steam or hot water, and provided with a mechanical stirrer revolving concentrically or otherwise. Fitting closely to the circular pan is a dome of about the same diameter and section as the lower pan. This dome has an aperture at its highest part, by which the vapors of the volatile solvent pass into an ordinary still-head which may surmount and form part of the dome, and thence to an ordinary condenser. The volatile solvent is driven off at the lowest possible temperature, and leaves the camphor disseminated in the solid or crystalline form throughout the grains or blocks, and even within the cell-walls of the nitro-cellulose. Up to this stage of the process the action of the solution of camphor upon the grains or blocks is inappreciable. The grains or blocks, through the entirety of whose mass finely-divided camphor has thus permeated, are now heated in a closed, though not necessarily air-tight, vessel at a temperature not higher than 100° centigrade. At this temperature the camphor exerts a remarkable action upon the nitro-cellulose, and the grains or blocks which at first were easily pliable are by this treatment rendered very hard, or of any required hardness, according to the percentage of camphor used in the solution. The camphor may now be driven out of the grains or blocks by sublimation or evaporation under ordinary or reduced pressures, or in a current of steam or air or other gas, or it may be washed out by treating the grains or blocks with any appropriate solvent or solvents of camphor.

When the apparatus mentioned above is used to effect the driving off of the volatile solvent, the whole of the operations—viz., mixing the grains or blocks with the solution of camphor, with or without the aforesaid exhaustion and readmission of air, driving off and condensing the volatile solvent, heating the grains or blocks containing solid camphor permeated through their mass, and, lastly, the driving off by heat and collecting the camphor driven off—may be conveniently carried out in the same apparatus.

When the camphor is to be removed from the blocks or grains by washing, a rapid process is to saturate the grains or blocks with some volatile solvent of camphor—such as light petroleum—and then expel the petroleum or other solvent with the camphor in solution by means of centrifugal force. With this object a centrifugal hydro-extractor, so constructed as to allow of as little air as possible passing through the grains or blocks, may be advantageously employed. Any slight residue of the volatile solvent left in the grains or blocks after the centrifugal process is expelled by means of heat. By varying the proportion of the camphor the action of the same upon the nitro-cellulose at and up to the temperature

named is such as to afford an exactly adjustable means of obtaining an explosive having any desired action or intensity, either sudden or more gradual, or even extremely gradual. It is to be distinctly understood that these results are obtained not by the presence of camphor in large or small quantities in the finished explosive, (from which most, if not all, the camphor has, on the contrary, been eliminated, as hereinbefore described,) but by a remarkable gelatinizing and, perhaps, some other action exerted by the camphor upon the nitro-cellulose when these are heated together at varying temperatures up to 100° centigrade, whereby the hardness and density of the explosive may be regulated at will by the proportion of camphor used.

Where conditions are such that an explosive is required of greater density than that obtained by the foregoing processes in the case of the grains treated as described, these are subjected *en masse* to a great pressure, so that a cake is formed. This cake is, however, easily broken up, practically, into the original grains, and these are found to possess a higher density, and have an angular or more or less flattened form, conducive to rapidity of ignition.

Instead of compressing the grains *en masse*, the grains may be passed between accurately-turned rollers, so adjusted as to exert a very considerable degree of pressure upon them, having the effect of increasing the density and giving a more or less angular or flattened form; or the hard approximately spherical granules may also, after treatment by the camphor process, be molded by compression into various forms—such as cylinders, prisms, cubes, or spheres. In this way small cylinders, for instance, containing the exact charge of powder for use in fire-arms, may be manufactured.

Instead of applying the compression to the hardened granules freed from camphor, as above, the granules freed from volatile solvent but still containing camphor permeating the mass, may be compressed or molded by compression. The forms—such as cylinders, prisms, cubes, or spheres—obtained by such compression are then heated at temperatures not exceeding 100° centigrade until the action of the camphor is complete and the camphor is finally removed, as far as practicable, either by sublimation or by being washed out by means of an appropriate solvent, as before described.

I claim—

1. The process, substantially as described, for the preparation of nitro-cellulose and compounds thereof for use as explosives, which consists in forming the same into grains or blocks, impregnating these with camphor by treatment with a solution of camphor in a volatile liquid not a solvent of nitro-cellulose, and expelling the solvent at a low temperature, then subjecting the camphorated nitro-cellulose to a temperature sufficiently high for the camphor to change the mechanical

of the nitro-cellulose, and finally expelling the camphor, all substantially as described.

2. The process, substantially as described; for the preparation of explosives, which consists in incorporating dinitro-cellulose with barium and potassium nitrates and carbon, treating the mixture with a solution of camphor in a volatile liquid not a solvent of dinitro-cellulose, evaporating the solvent at a low

temperature, then subjecting the camphorized material to a temperature sufficiently high for the camphor to change the mechanical state of the dinitro-cellulose, and finally expelling the camphor, all substantially as described.

DAVID JOHNSON.

Witnesses:

C. A. JENSEN,

WALTER J. SKERTEN.